

# United States Patent Office

3,033,704

Patented May 8, 1962

1

3,033,704

## RENDERING FABRIC ANTI-STATIC, SOFT, AND MICROORGANISMS RESISTANT

Joseph C. Sherrill, Park Forest, Warner M. Limfield, Evanston, and Byron E. Marsh, Brookfield, Ill., assignors, by mesne assignments, to Armour and Company, Chicago, Ill., a corporation of Delaware  
No Drawing. Filed May 19, 1959, Ser. No. 814,149  
3 Claims. (Cl. 117—47)

This invention relates to a novel laundering process, and more particularly to a special treatment which renders fabrics substantially anti-static and soft and at least partially free from microorganisms.

The use of cationic surface active agents as a fabric softener and to render fabrics anti-static and substantially free from lint is well known. However, cationic surface active agents are only minimally effective as antibacterial agents. On the other hand, effective antibacterial agents such as organomercurials are only minimally substantive to fabrics. Thus, although methods are known for rendering fabrics soft, anti-static and substantially lint-free by the treatment thereof with cationic surface active agents, the provision of fabrics also at least partially free from microorganisms in a laundering process has not as yet been satisfactorily obtained.

Accordingly, it is an object of this invention to provide a laundering process in which a fabric is rendered substantially anti-static and lint-free and soft, while at the same time rendering the fabric at least partially free from microorganisms. Other advantages will become apparent as the specification proceeds.

In the special treatment of this invention the fabric is impregnated with a mixture of at least one cationic surface active agent and at least one organomercurial germicide to render such fabric substantially anti-static and soft and at least partially free from microorganisms.

In a preferred aspect of this invention, treatment of the fabrics is obtained in a laundering process in which a laundered fabric is contacted in a rinsing operation with an aqueous solution of a mixture of at least one cationic surface active agent and at least one organomercurial germicide to impregnate the fabric with at least a portion of the organomercurial and the cationic surface active agent, and in which the treated fabric is then at least substantially dehydrated.

Although the advantages of this invention may be achieved with any cationic surface active agent, better results are obtained with a cationic surface active agent of the group having the formulae



and



and



(3)

wherein  $R_1$  is an alkyl radical containing from 10 to 22 carbon atoms, wherein  $R_2$  represents a benzyl radical or an alkyl radical containing less than 3 carbon atoms, wherein  $R_3$  is an alkyl radical containing less than 3 carbon atoms, and wherein  $X$  represents an anion of the group consisting of chloride, bromide, sulfate and an alkyl sulfate in which the alkyl radical contains less than 5 carbon atoms. Furthermore, the alkyl group repre-

2

sented by  $R_1$  in the above formulae may be a natural mixture thereof derived from tallow, soybean or coconut oil. Also, it is known that cationic surface active agents which include a greater number of the long-chain alkyl groups demonstrate better fabric softening properties, whereas a greater number of short-chain alkyl groups included in the cationic surface active agent tends towards better germicidal activity. Accordingly, compounds having the Formula 1 above tend toward greater germicidal activity than those having the Formula 2 above, whereas compounds having the Formula 2 tend toward greater fabric-softening action than those having the Formula 1 above. Even better results may be obtained with cationic surface active agents having Formulae 1 and 2 above in which  $R_1$  represents an alkyl radical containing from 12 to 18 carbon atoms, wherein  $R_2$  is a benzyl radical, wherein  $R_3$  is a methyl radical, and wherein  $X$  is chloride.

Although any organomercurial germicide may be employed in the treatment of this invention, better results are obtained with phenylmercuric compounds such as the acetate, propionate, butyrate, chloride, bromide or iodide thereof.

In the preferred practice of this invention fabrics, after laundering, are immersed in a rinse water containing a mixture of at least one cationic surface active agent and at least one organomercurial germicide in which mixture the organomercurial is included in a ratio of from 1 to 10% by weight of the cationic surface active agent, and in which the cationic surface agent is included in a ratio of from 0.03 to 0.3% by weight of the fabric. After the fabric has been impregnated with at least a portion of the mixture of the organomercurial and the cationic surface active agent, the fabric is at least substantially dehydrated.

Although the advantages of this invention may be obtained by employing from 1 to 10% of the organomercurial in combination with the cationic surface active agent, better results are obtained with a ratio of organomercurial of from 4 to 8% by weight of the cationic surface active agent. Especially desirable for utilization in this invention is a mixture of about 5.5 to 6% by weight of the organomercurial in combination with the cationic surface active agent.

Although the ratio of cationic surface active agent to fabric employed in this invention may be from 0.03 to 0.3% by weight, better results are obtained at a ratio of 0.065 to 0.1% by weight of cationic surface active agent in contact with the fabric. Furthermore, it has been found that from 0.03 to 0.065% by weight of cationic surface active agent in combination with the fabric facilitates pressing operations by rendering the fabric easier to handle, whereas tactile softness is achieved especially at a ratio of 0.065 to 0.1% by weight of cationic surface active agent in combination with the fabric. Accordingly, especially desirable in the treatment of this invention is a ratio of about 0.1% by weight of the cationic surface active agent in combination with the fabric.

The ratio of organomercurial to fabric employed in this process may be from 7 to 70 p.p.m. Although optimal results have been achieved at a ratio of organomercurial to fabric of about 60 p.p.m., satisfactory results may be obtained at a ratio of about 43 p.p.m. of organomercurial in combination with the fabric.

It is anticipated that a mixture of at least one cationic surface active agent and at least one organomercurial germicide can be packaged in the aforementioned ratio to be employed in laundering plants by introduction into a rinse water at the hereinbefore described concentration. After the rinsing operation has been completed, the fabrics can be separated from the bulk of the rinse water, and then subjected to dehydration.

This invention is further illustrated in the following specific examples:

3  
*Example I*

The following formulation has been employed in the treatment of this invention:

| Ingredient                                          | Concentration |                |
|-----------------------------------------------------|---------------|----------------|
|                                                     | Percent total | Percent active |
| Softener 2-132 (75%) <sup>1</sup>                   | 13.40         | 10.0           |
| Arquad-S <sup>2</sup> (50%)                         | 10.00         | 5.0            |
| Phenylmercuric propionate                           | 0.85          | 0.85           |
| Hexylene glycol                                     | 2.00          |                |
| Sodium sulfate                                      | 0.20          |                |
| Hidacid blue V, conc. No. 20-2214 (1%) <sup>3</sup> | 0.50          |                |
| Brightener: Uvitex SN (10%) <sup>4</sup>            | 0.38          |                |
| Water                                               | 72.67         |                |
| Perfume <sup>5</sup>                                | 0.125         |                |

<sup>1</sup> This is a cationic surface active agent having formula (3) above in which the alkyl radicals represented by R<sub>1</sub> are derived from tallow, soybean or coconut fatty acids, in which R<sub>2</sub> represents an alkyl radical containing less than 3 carbon atoms, and in which X represents methyl sulfate.

<sup>2</sup> Arquad-S. This is a cationic surface active agent having the formula (1) above in which the alkyl radical represented by R<sub>1</sub> is derived from tallow fatty acids, in which R<sub>2</sub> and R<sub>3</sub> represent methyl radicals, and in which X represents chloride.

<sup>3</sup> This is a dye of the pigment group.

<sup>4</sup> This is an optical brightener of the arylimidazole type.

<sup>5</sup> Any perfume may be employed in this type of formulation, which perfumes are well-known and widely used.

In preparing this formulation, the phenylmercuric propionate is first wetted and finely dispersed in the hexylene glycol so that no lumps remain. This dispersion is thoroughly mixed with melted Softener 2-132 which has been preheated to a temperature of about 140 to 150° F. the resulting mixture is added slowly, with agitation, to the water and dye solution which has been heated to a temperature of about 120 to 130° F. As the melted softener-organomercurial dispersion is added to the solution the viscosity of the mix will increase gradually due to gel formation. The viscosity of the mixture should be permitted to rise as high as the mixing equipment allows, and thereafter the viscosity is controlled by the addition to the mixture of small increments of the sodium sulfate. After the batch has been uniformly blended, the Arquad-S may be slowly added to the mixture at room temperature, whereupon a reduction in viscosity will be obtained. Thereafter the brightener and perfume are added to the mixture, and agitation thereof is continued until the mass has become homogeneous. However, prolonged agitation after addition to the mixture of the brightener is not desirable. After the mixing has been completed, the batch should be processed through a colloid mill or homogenizer.

The foregoing sequence of addition of the ingredients is important in that the premixing of the cationic surface active agents, namely the Softener 2-132 and the Arquad-S, results in a relatively high concentration of chloride ion in the acidic medium, and consequently agglomeration of the phenylmercuric propionate in the mixture, which agglomeration is difficult to disperse.

This formulation may be introduced into the rinse water on the basis of 12 fluid ounces per one hundred pounds of fabric. Accordingly, there will be obtained in the rinse water 0.111% of the cationic surface active agent in combination with the fabric. Also, there will be obtained with this formulation in the rinse water about 63 p.p.m. of phenylmercuric propionate in combination with the fabric.

*Example II*

There may be employed in the rinsing process of this invention the formulation of Example I in which, instead of the mixture of Softener 2-132 and Arquad-S specified in the formulation thereof, 20% of Softener 2-132 is utilized. Accordingly, there will be provided in the formulation 15% of "active" Softener 2-132.

4  
*Example III*

There may be employed in the rinsing process of this invention the formulation of Example I in which, instead of the mixture of Softener 2-132 and Arquad-S, 20% of Arquad 2HT (75%) is substituted. Accordingly, the formulation will include 15% of "active" Arquad 2HT. Arquad 2HT is a cationic surface active agent having the Formula 2 above in which the alkyl radicals represented by R<sub>1</sub> are derived from partially hydrogenated tallow fatty acids, in which R<sub>2</sub> and R<sub>3</sub> represent methyl radicals and in which X is chloride.

*Example IV*

15 There may be employed in the rinsing process of this invention the formulation of Example I in which, instead of phenylmercuric propionate, 0.85% of phenylmercuric acetate is substituted.

*Example V*

There may be employed in the rinsing process of this invention the formulation of Example I in which, instead of the mixture of Softener 2-132 and Arquad-S, a mixture of 13.40% of Arquad 2HT (75%) and 10.00% of Arquad-S is substituted. Accordingly, there will be included in the formulation 10.0% of "active" Arquad 2HT and 5.0% of "active" Arquad-S.

*Example VI*

There may be employed in the rinsing process of this invention the formulation of Example I in which, instead of the Softener 2-132 and Arquad-S and phenylmercuric propionate, 13.40% of Arquad 2HT and 10.00% of Arquad-S and 0.85% of phenylmercuric acetate is substituted. Accordingly, there will be included in the formulation 10.0% of "active" Arquad 2HT and 5.0% of "active" Arquad-S.

*Example VII*

40 There may be employed in the rinsing process of this invention the formulation of Example I in which, instead of the mixture of Softener 2-132 and Arquad-S and phenylmercuric propionate, 20.00% of Softener 2-132 and 0.85% of phenylmercuric acetate is substituted. Accordingly, there will be included in the formulation 15.00% of "active" Softener 2-132.

*Example VIII*

50 There may be employed in the rinsing process of this invention the formulation of Example I in which, instead of Softener 2-132, 10.0% active of a cationic surface active agent having Formula 2 above in which the alkyl radicals represented by R<sub>1</sub> contain 12 carbon atoms, in which R<sub>2</sub> and R<sub>3</sub> represent methyl radicals, and in which X represents chloride. Also, instead of phenylmercuric propionate, 0.85% phenylmercuric chloride is substituted. The pH of the formulation is adjusted to an alkaline level with an alkaline salt or an alkali. Accordingly, there will be included in the formulation 10.0% "active" of 60 the above described cationic agent and 5.0% "active" Arquad-S.

*Example IX*

65 There may be employed in the rinsing process of this invention the formulation of Example I in which, instead of a mixture of Softener 2-132 and Arquad-S, 10.0% active of a cationic agent having Formula 3 above in which R<sub>1</sub> is an alkyl radical containing 12 carbon atoms, in which R<sub>3</sub> is a methyl radical, and in which X represents chloride, 5.0% active of a cationic agent having Formula 1 above with the substitution therein being the same as for Arquad-S with the exception that X represents chloride instead of methyl sulfate. Also 0.85% phenylmercuric butyrate is substituted for the phenylmercuric propionate specified in the formula of Example I.

5  
*Example X*

There may be employed in the rinsing process of this invention the formulation of Example I in which is substituted, instead of a mixture of Softener 2-132 and Arquad-S, 15% active of a cationic agent having the Formula 3 above in which R<sub>1</sub> represents alkyl radicals derived from tallow, soybean or coconut fatty acids, in which R<sub>3</sub> is a benzyl radical, and in which X represents chloride, is substituted.

10  
*Example XI*

There may be employed in the rinsing process of this invention the formulation of Example I in which is substituted, instead of a mixture of Softener 2-132 and Arquad-S, 15% active of a cationic agent having the Formula 3 above in which R<sub>1</sub> represents alkyl radicals containing 22 carbon atoms, in which R<sub>3</sub> represents a methyl radical, and in which X represents phenylsulfonate or benzylsulfonate.

20  
*Example XII*

There may be employed in the rinsing process of this invention the formulation of Example I in which is substituted, instead of a mixture of Softener 2-132 and Arquad-S, 15% active of a cationic agent having the Formula 3 above in which R<sub>1</sub> is an alkyl radical containing 10 carbon atoms, in which R<sub>3</sub> represents a methyl radical and in which X represents phenylsulfonate or benzylsulfonate. Also, there is substituted for the phenylmercuric propionate therein, 0.85% of phenylmercuric butyrate.

25  
*Example XIII*

There may be employed in the rinsing process of this invention the formulation of Example I in which is substituted, instead of a mixture of Softener 2-132 and Arquad-S, 15% active of a cationic agent having the Formula 1 above in which R<sub>1</sub> is an alkyl radical containing 10 to 22 carbon atoms derived from tallow, soybean or coconut fatty acids, in which R<sub>2</sub> represents a benzyl radical, in which R<sub>3</sub> is a methyl radical, and in which X represents a chloride ion. Also, instead of phenylmercuric propionate, 0.85% of phenylmercuric acetate is substituted.

30  
*Example XIV*

There may be employed in the rinsing process of this invention the formulation of Example I in which is substituted, instead of a mixture of Softener 2-132 and Arquad-S, 13.40% of Arquad 2HT (75%) and 5.0% active of a cationic agent having the formula



wherein R<sub>1</sub> is an alkyl radical containing 12 carbon atoms and wherein X represents chloride or bromide. Accordingly, the formulation will include 10.0% of "active" Arquad 2HT and 5.0% of "active" alkyl pyridinium halide described above.

35  
*Example XV*

There may be employed in the rinsing process of this invention the formulation of Example I in which is substituted, instead of Arquad-S and phenylmercuric propionate, 5.0% active of a cationic agent having the formula of Example XIII wherein R<sub>1</sub> is an alkyl radical having 18 carbon atoms and wherein X represents a chloride or bromide anion and 0.85% phenylmercuric butyrate. Accordingly, the formulation will include 10.0% of "active" Softener 2-132 and 5.0% of "active" alkyl pyridinium halide described above.

6  
*Example XVI*

There may be employed in the rinsing process of this invention the formulation of Example I in which is substituted, instead of a mixture of Softener 2-132 and Arquad-S, 15.0% active of a cationic agent having the formula



15 wherein R<sub>1</sub> is an alkyl radical containing 10 carbon atoms, wherein R<sub>2</sub> is an ethanol radical, wherein R<sub>3</sub> is a methyl radical, and wherein X represents methyl sulfate. Also, instead of phenylmercuric propionate, phenylmercuric acetate is substituted.

20  
*Example XVII*

There may be employed in the rinsing process of this invention the formulation of Example I in which is substituted, instead of a mixture of Softener 2-132 and Arquad-S and phenylmercuric propionate, 15.0% active of a cationic agent having the formula of Example XVI wherein R<sub>1</sub> is an alkyl radical containing 22 carbon atoms, wherein R<sub>2</sub> is an ethanol radical, wherein R<sub>3</sub> is a methyl radical, and wherein X is phenyl sulfonate or benzyl sulfonate, and 0.85% phenylmercuric butyrate.

25  
*Example XVIII*

There may be employed in the rinsing process of this invention the formulation of Example I in which is substituted, instead of Softener 2-132 and Arquad-S, 13.40% of Arquad 2HT (75%) and 5.0% active of a cationic agent having the formula of Example XV wherein R<sub>1</sub> is an alkyl radical containing 10 to 22 carbon atoms derived from tallow, soybean or coconut fatty acids, in which R<sub>2</sub> is an ethanol radical, wherein R<sub>3</sub> is a benzyl radical, and wherein X represents a chloride anion.

30  
*Example XIX*

There may be employed in the rinsing process of this invention the formulation of Example I in which is substituted, instead of Softener 2-132 and Arquad-S and phenylmercuric propionate, 13.4% of Arquad 2HT (75%) and 5.0% active of a cationic agent of the type "Hyamine 1622" (Rohm and Haas) and 0.85% phenylmercuric acetate. Accordingly, the formulation will include 100% of "active" Arquad 2HT and 5.0% of active "Hyamine 1622."

35  
*Example XX*

There may be employed in the rinsing process of this invention the formulation of Example I in which is substituted, instead of Arquad-S, 5.0% active of a cationic agent of the type "Emcol E-607."

40  
*Example XXI*

There may be employed in the rinsing process of this invention the formulation of Example I in which is substituted, instead of Softener 2-132 and Arquad-S and phenylmercuric propionate, 13.40% of Arquad 2HT (75%) and 5.0% "active" of a cationic agent of the type "Emcol E-11" and 0.85% phenylmercuric acetate. Accordingly, the formulation will include 10.0% of "active" Arquad 2HT and 5.0% of "active" "Emcol E-11."

45  
*Example XXII*

There may be employed in the rinsing process of this invention the formulation of Example I in which is substituted, instead of Arquad-S, 5% active of a cationic agent of the type "Emcol E-11." Accordingly, the formulation will include 10.0% of "active" Softener 2-132 and 5.0% of "active" "Emcol E-11."

7  
*Example XXIII*

There may be employed in the rinsing process of this invention the formulation of Example I, except that 0.36 instead of 0.8% phenylmercuric propionate is used. This formulation is utilized in the rinsing process on the basis of  $\frac{3}{4}$  liquid ounces per one hundred pounds of fabric. Accordingly there will be obtained in the rinse water 0.03% of the cationic surface active agent in combination with the fabric. Also, there will be obtained with this formulation in the rinse water about 7 p.p.m. of phenylmercuric propionate in combination with the fabric.

8  
*Example XXIV*

There may be employed in the rinsing process of this invention the formulation of Example XXII, except that  $32\frac{1}{2}$  fluid ounces are used per 100 pounds of fabric. Accordingly there will be obtained in the rinse water 0.3% of the cationic surface active agent in combination with the fabric. Also, there will be obtained with this formulation in the rinse water about 70 p.p.m. phenylmercuric propionate in combination with the fabric.

15  
*Example XXV*

There may be employed in the rinsing process of this invention the formulation of Example I, except that 0.15 instead of 0.85% phenylmercuric propionate is used. This formulation is used on the basis of  $7\frac{1}{2}$  fluid ounces per one hundred pounds of fabric. Accordingly there will be obtained in the rinse water 0.07% of the cationic surface active agent in combination with the fabric. Also, there will be obtained with this formulation in the rinse water about 7 p.p.m. of phenylmercuric propionate in combination with the fabric.

20  
*Example XXVI*

There may be employed in the rinsing process of this invention the formulation of Example I, except that 1.5 instead of 0.85% phenylmercuric propionate is used. This formulation is used on the basis of  $7\frac{1}{2}$  fluid ounces per one hundred pounds of fabric. Accordingly there will be obtained in the rinse water 0.07 of the cationic surface active agent in combination with the fabric. Also there will be obtained with this formulation in the rinse water about 70 p.p.m. phenylmercuric propionate in combination with the fabric.

25  
*Example XXVII*

The enhanced impregnation of the fabric with the organomercurial, and the consequent increased antibacterial effect, obtained by the treatment of this invention, can be demonstrated as follows:

In this comparison, the cationic surface active agent, quaternized imidazoline, was included in a rinse water at a ratio of 0.079% by weight of the fabrics, while phenylmercuric propionate was included in the rinse water at a concentration of 50 p.p.m. of the fabric.

In one process of this comparison, the fabrics were first treated in rinse water with the cationic surface active agent, and, after draining the first rinse water, a second rinse water containing the phenylmercuric propionate was contacted with the fabric. The results were as follows:

|               | Concentrations, OWF <sup>1</sup> |                    | Staphylococcus aureus (FDA Strain No. 209), zones of inhibition (mm.) |    |   |   |      |
|---------------|----------------------------------|--------------------|-----------------------------------------------------------------------|----|---|---|------|
|               | Cationic (percent)               | Mercurial (p.p.m.) | 1                                                                     | 2  | 3 | 4 | Avg. |
|               |                                  |                    | Experiment 1a                                                         | 50 | 5 | 4 | 1    |
| Experiment 1b | 0.079                            | 50                 | 5                                                                     | 4  | 1 | 3 | 3    |

<sup>1</sup> On weight of fabric.

In a second process, a mixture of the cationic surface active agent and the phenylmercuric propionate was in-

duced into a single rinse water which was contacted with the fabrics. The results were as follows:

| 10            |               | Concentrations, OWF <sup>1</sup> |                    | Staphylococcus aureus (FDA Strain No. 209), zones of inhibition (mm.) |   |   |   |      |
|---------------|---------------|----------------------------------|--------------------|-----------------------------------------------------------------------|---|---|---|------|
|               |               | Cationic (percent)               | Mercurial (p.p.m.) | 1                                                                     | 2 | 3 | 4 | Avg. |
|               | Experiment 2a | 0.079                            | 50                 | 5                                                                     | 7 | 7 | 6 | 6    |
| Experiment 2b | 0.079         | 50                               | 5                  | 6                                                                     | 7 | 5 | 6 | 6    |

<sup>1</sup> On weight of fabric.

15 In the foregoing, the evaluation of the treated fabric was obtained by introducing a portion of the fabric on seeded agar plates which were incubated at a temperature of  $98.6^{\circ}$  F. for a period of 24 hours. The term "zones of inhibition" refers to the width in mm. of no-growth areas of agar surrounding the treated fabric.

20 These results indicate that a greater amount of phenylmercuric propionate is impregnated in the fabric when a mixture of the phenylmercuric propionate and the cationic surface active agent is contacted with the fabric in comparison with the treatment of the fabric with separate rinses of the cationic surface active agent and of the phenylmercuric propionate, and consequently that a greater anti-bacterial effect is thereby obtained.

25 Instead of the phenylmercuric propionate and phenylmercuric acetate specified in the formulations of these examples, there may be employed as the organomercurial in this rinsing process phenylmercuric chloride, bromide, iodide and butyrate.

30 The FDA strain No. 209 of *S. aureus* is a standard microorganism employed in experimentation. It has been found that zones of inhibition against this organism in the order of 3-5 mm. results in a minimal effect against 35 resistant strains of *S. aureus*, and that similar zones of inhibition represent minimal effects against ammonia-producing microorganisms. On the other hand, it has been shown that zones of inhibition in the order of 7-12 mm. indicate effectiveness against resistant strains of *S. aureus*. Consequently, it will be seen that the treatment of this invention results in the impregnation of the fabric with an amount of the organomercurial adequate to obtain inhibition of growth of resistant strains of *S. aureus*, whereas the treatment of the fabric with separate rinses of the cationic surface active agent and of the organomercurial provide impregnation of the fabric with the organomercurial in such concentration as to provide inhibition of these resistant strains.

35 While in the foregoing specification various embodiments of this invention have been illustrated in considerable detail for the purpose of illustration, it will be apparent to those skilled in the art that this invention is susceptible to other embodiments and that many of these details can be varied widely without departing from the basic concept and spirit of the invention.

40 We claim:

45 1. In a laundering and fabric-softening process, the steps of rinsing a laundered fabric in an aqueous solution of a mixture of at least one cationic surface active agent and at least one organomercurial germicide, said organomercurial germicide being included in said mixture in a ratio of from 1 to 10% by weight of said cationic surface active agent, and said cationic surface active agent being employed in a ratio of from 0.03 to 50 0.3% by weight of said fabric, to impregnate said fabric with at least a portion of said organomercurial germicide and said cationic surface active agent, and then at least substantially dehydrating said fabric.

55 2. In a laundering process for softening fabrics, the steps of rinsing a laundered fabric in an aqueous solution

of a mixture of at least one phenylmercuric compound and at least one cationic surface active agent selected from the group having the formula

and  $[R_1NR_2(R_3)_2]^+ X^-$  and  $[(R_1)_2NR_2R_3]^+ X^-$



wherein R<sub>1</sub> represents an alkyl radical containing from 10 to 22 carbon atoms, wherein R<sub>2</sub> is selected from the group consisting of a benzyl radical and an alkyl radical containing less than 3 carbon atoms, wherein R<sub>3</sub> represents an alkyl radical containing less than 3 carbon atoms and wherein X is an anion selected from the group consisting of chloride, bromide, sulfate and an alkyl sulfate in which the alkyl radical contains less than 5 carbon atoms, said phenylmercuric compound being included in said mixture in a ratio of from 4 to 8% by weight of said cationic surface active agent, and said cationic surface active agent being employed in a ratio of from 0.065 to 0.1% by weight of said fabric, to impregnate said fabric

with at least a portion of said phenylmercuric compound and said cationic surface active agent, and then at least substantially dehydrating said fabric.

3. Treatment to render fabrics substantially anti-static  
5 and soft and at least partially free from microorganisms  
by rinsing a fabric in an aqueous solution containing at  
least one cationic surface active agent and at least one  
organomercurial germicide to impregnate the fabric with  
at least a portion of said cationic surface active agent and  
10 said organomercurial germicide, and then at least sub-  
stantially dehydrating said fabric, said organomercurial  
germicide being employed in a ratio of from 1 to 10% by  
weight of said cationic surface-active agent.

**References Cited** in the file of this patent

UNITED STATES PATENTS

|           |             |               |
|-----------|-------------|---------------|
| 2,423,261 | Sowa        | July 1, 1947  |
| 2,536,750 | Kamlet      | Jan. 2, 1951  |
| 2,734,830 | Hagge et al | Feb. 14, 1956 |
| 2,898,262 | Dietz       | Aug. 4, 1959  |

## FOREIGN PATENTS

605,442 Great Britain ..... July 23, 1948  
132,125 Australia ..... Apr. 11, 1949